

# United States Patent Office

3,827,894

Patented Aug. 6, 1974

## 1

3,827,894  
**CEMENTITIOUS COATING CONTAINING  
 NON-ABRASIVE FILLER**  
 Howard C. Hansen, 926 E. Hermosa Drive,  
 Tempe, Ariz. 85281  
 No Drawing. Filed Dec. 13, 1972, Ser. No. 314,863  
 Int. Cl. C04b 7/08

U.S. CL 106—90

11 Claims

## ABSTRACT OF THE DISCLOSURE

A protective coating for concrete, slate and gravel covered roof structures prepared from a preferred mixture comprising: white cement, white waterproof cement, non-abrasive fillers, a whitening agent, a setting agent, a binder, and water.

## BACKGROUND OF THE INVENTION

### Field of the Invention

This invention relates to coating products and more particularly to a coating product for use on concrete, slate or gravel covered roof structures.

### Description of the Prior Art

Many roof coating products are available from numerous suppliers and these prior art products are of various formulations depending on regional climate conditions, cost of the ingredients, type of roof structure and the like.

In relatively warm climates roof coatings are normally white in color for optimum reflectivity and thus minimum heat transfer. Prior art roof coatings generally employ a portland cement of the usual gray color and depend entirely on chemical whiteners to obtain the desired degree of whiteness.

Prior art roof coating of the above type are subject to relatively rapid discoloration due to the iron oxide content of the portland cement used in their mixture, and thus a reduction in the reflectivity occurs as the discoloration progresses.

Many of the prior art roof coatings generally employed are subject to water caused deterioration and will not withstand much in the way of externally applied forces. For example, a gravel roof is particularly susceptible to these problems as may be evidenced by the loss of gravel resulting from a rain storm and by the gravel being kicked loose when a person walks on the roof.

When roof coating products are commercially applied, they are usually applied in at least two successive coats which are sprayed with suitable apparatus.

Many of the prior art products contain a sand filler which causes rapid destruction of the spraying equipment due to the abrasive nature of the sand.

The setting time between successive coats is of prime importance to a contractor due to the high cost of labor and the necessity of returning to a job site if this time is excessive. Thus, most of the available products contain a chemical accelerator to speed up the set time. However, most producers of this type of product do not take into account the variations in relative humidity which largely determines the set time. Hence, the producers add a fixed amount of the accelerator to their product and the contractor must live with large variations in setting time as determined by variations in humidity.

In view of the above, it may be seen that a need exists for a roof coating product which overcomes some of the limitations of the prior art.

## 2

## SUMMARY OF THE INVENTION

In accordance with the present invention a new and useful roof coating product is disclosed for use on concrete, slate, and gravel covered roof structures.

5 The product of the instant invention includes a preferred mixture of two white cements which provide the product with strength, resistance to water caused deterioration, and have a natural whiteness; thus, the discoloration which occurs in prior art mixtures does not occur in this mixture.

Some of the whiteness of the present product is derived from the inclusion of the white cements as hereinbefore described, and this whiteness is enhanced by the addition of a whitening agent.

15 A non-abrasive filler material is used in the present mixture to reduce damage to the applicating equipment.

The above elements are mixed into a homogeneous compound which is shipped to the job site in dry form. Preparation of this product for use includes the addition of a binder, a chemical accelerator and water. The amount of accelerator used is determined at the job site with humidity at that specific location and time being the determining factor.

20 Accordingly, it is an object of the present invention to provide a new and useful roof coating product for use on concrete, slate and gravel covered roof structures.

Another object of the present invention is to provide a new and useful roof coating product which is strong, resists water caused deterioration and resists discoloration.

25 Another object of the present invention is to provide a new and useful roof coating mixture which employs non-abrasive filler material to prolong the life of applicating equipment.

30 Still another object of the present invention is to provide a new and useful roof coating product of the above described character the setting time of which is controlled by adding a chemical accelerator thereto at the time of use in quantity determined by the relative humidity at that specific time and location.

35 The foregoing and other objects of this invention, as well as the invention itself, may be more fully understood from the following description of the preferred embodiment.

## DESCRIPTION OF THE PREFERRED EMBODIMENT

The roof coating product of the present invention is a mixture of various ingredients which provide various 40 desirable characteristics as will be described in detail, with one of these characteristics being a coating which is white in color and will not discolor with age. The white color is particularly desirable in warm climates due to its high reflectivity which provides a low heat transfer characteristic to the present product.

45 The desired white color of the product of the present invention and its resistance to discoloration is derived from two ingredients. The first ingredient is the cement and the second is a whitening agent.

50 The cement is preferably a mixture of two types of cement which are referred to as white cements. As is well known in the art, white cement is a portland cement which does not contain any iron oxide and thus is white in color.

55 The first of these cements is white cement having what is commonly called high-early strength. High-early strength white cement differs from conventional cement in that it sets more rapidly.

60 The second of these cements is white cement containing well known additives which render it waterproof.

65 The mixture of the above described white cements not only provides a natural whiteness and waterproof char-

acteristics to the present product, it also provides a rapidly achieved high resistance to externally applied forces. The resistance to externally applied forces will vary from manufacturer to manufacturer according to their particular formula. Thus, a cement having a high-early strength in the range of about 1,000 p.s.i. is preferred.

The mix ratio of the above described white cements may be allowed to vary somewhat in accordance with the desired degree of resistance to water caused deterioration and the desired rapidity of obtaining the high-early strength. If in a particular application obtaining high-early strength is of prime importance, the amount of high-early white cement employed should be increased with a proportionate decrease in the amount of white waterproof cement. If resistance to water caused deterioration is important in a particular application, the above mentioned increase and decrease in the quantities of the two cements should be reversed. The preferred mix ratio of the two cements is in the amount of about  $\frac{1}{2}$  high-early white cement and about  $\frac{1}{2}$  white waterproof cement. It has been determined that excessive deviations of the above preferred mix ratio can cause undesirable results, i.e., if the product sets too fast, cracking may result, and if it sets too slowly, excessive time between coatings occurs.

A whitening agent is added to the above mixture of cements to augment the natural whiteness provided by the hereinbefore described white cement and white waterproof cement. The preferred product employed as the whitening agent is titanium which is a dark gray, lustrous, metallic element in its natural state. As is well known, the basic element titanium may be processed into titanic oxide, sometimes known as titanic dioxide,  $TiO_2$ , which is a white crystalline compound often used as a pigment.

Also added to the above mixture of two cements is a non-abrasive filler such as talc. The non-abrasive characteristics of the filler is important so that damage to applying equipment, such as spray apparatus, may be held to a minimum.

It is noted that the mixture of the two cements, the whitening agent and the non-abrasive fillers as thus far described, is a dry powder formulation. This formulation is thoroughly mixed into a homogenous compound which is shipped from the manufacturing location to a job site in this form.

At the job site a binder, a chemical accelerator, or setting agent and water are added to the dry formulation in predetermined quantities and thorough mixing at this time is important to provide an easily applicable product of consistant quality and characteristics.

The binder employed may be any suitable well known binder such as epoxy, a silicate of soda solution and the like. However, the preferred binder is a polyvinyl acetate emulsion as is commonly used in roof coatings of this type.

The water added at the time of use should for obvious reasons be of tap or drinking water purity to prevent unfavorable reactions and/or discoloration.

The chemical accelerator, or setting agent, which may be employed to control the setting time of the coating, will also determine the pot-life or working time of the product.

In the art, the term "pot-life" or "working time" refer to that period of time between the formation of a wet mix and the solidification thereof into an unworkable mass, that is, a mass which can no longer be applied to a roof structure. The term "setting time" refers to that period of time between the application of a first coat and the application of a second coat.

The setting agent employed in the roof coating of the present invention is calcium chloride, but it is not intended that this specific compound be construed as a limitation to the present invention as it should be understood that other well known setting agents could be employed, such as magnesium chloride and the like.

As is well known, relative humidity is a prime factor which effects the setting time in applications of coatings

of this nature. Therefore, the coating of the present invention ideally includes the addition of the setting agent in various amounts as determined by the humidity reading at a specific job site.

By way of example, assume that a particular job site has a humidity reading of 20%, and that  $\frac{1}{8}$  part per weight of the setting agent added to a specific quantity of the mix of the present invention will result in a pot-life of 45 minutes and a setting time of between one and two hours. It should be noted that the setting time mentioned above will vary somewhat with the thickness of the coating, thus the above time is predicated on a thickness resulting from an application of about two (2) gallons per 100 sq. ft. which is average for at least the first application of a coating of this type.

Should it be desired that all the above parameters remain the same in an instance where the humidity reading is 30%,  $\frac{3}{16}$  parts by weight of the setting agent would be needed to hold the pot-life and setting time substantially the same. Thus, it may be stated that with the above parameters, that about  $\frac{1}{16}$  part by weight is needed for each 10% of relative humidity.

It should be noted that the addition of the setting agent may be omitted from the present invention when the relative humidity at a particular locale is low, that is, readings up to about 40%, without serious effects to the pot-life and setting time. However, at readings from about 40% and up the setting agent becomes very important.

The ingredients employed in the preparation of the product of the present invention are generally within the following proportions:

| Ingredient:         | Parts by weight                |
|---------------------|--------------------------------|
| Whitener            | 2 to 3                         |
| Non-abrasive filler | 8 to 11                        |
| White cement        | 34 to 42                       |
| Setting agent       | $\frac{1}{8}$ to $\frac{1}{2}$ |
| Binder              | 7 to 9                         |
| Water               | 75 to 85                       |

The preferred mix and range of proportions is:

| Ingredient:                       | Parts by weight                                        |
|-----------------------------------|--------------------------------------------------------|
| Titanic oxide                     | 2 to 3.                                                |
| Talc                              | 8 to 11.                                               |
| High-early strength white cement. | 17 to 21.                                              |
| White waterproof cement           | 17 to 21.                                              |
| Calcium chloride                  | $\frac{1}{16}$ part for each 10% of relative humidity. |
| Polyvinyl acetate emulsion        | 7 to 9.                                                |
| Water                             | 75 to 85.                                              |

While the principles of the invention have now been made clear in an illustrated embodiment, there will be immediately obvious to those skilled in the art, many modifications of proportions, the elements, materials, and compounds used in the practice of the invention, and otherwise, which are particularly adapted for specific environments and operation requirements without departing from those principles. The appended claims are therefore intended to cover and embrace any such modifications within the limits only of the true spirit and scope of the invention.

What I claim is:

1. A coating composition for use on concrete, slate and gravel covered roof structures, said composition prepared from a mix comprising in combination: a whitening agent; non-abrasive fillers in the form of talc; white cement; a binding agent; and water.
2. A coating composition as claimed in Claim 1 where-in said white cement includes a mixture of high-early strength white cement and white waterproof cement.
3. A coating composition as claimed in Claim 1 where-in said white cement includes a mixture of approximately

$\frac{1}{2}$  high-early strength white cement and approximately  $\frac{1}{2}$  white waterproof cement.

4. A coating composition as claimed in Claim 1 wherein said whitening agent is titanium processed to form titanic oxide.

5. A coating composition as claimed in Claim 1 wherein said binder includes a polyvinyl acetate emulsion.

6. A coating composition as claimed in Claim 1 further including a setting agent.

7. A coating composition as claimed in Claim 6 wherein said setting agent is added in quantities of approximately  $\frac{1}{16}$  part by weight for each 10% of relative humidity as determined by the relative humidity reading at the specific location and time of use.

8. A coating composition as claimed in Claim 6 wherein said setting agent includes calcium chloride.

9. A coating composition for use on concrete, slate and gravel covered roof structures, said composition prepared from a mix comprising in combination:

(a) a whitening agent in an amount of about 2 parts by weight to 3 parts by weight;

(b) non-abrasive fillers in the form of talc in an amount of about 8 parts by weight to about 11 parts by weight;

(c) white cement in the amount of about 34 parts by weight to about 42 parts by weight;

(d) a binding agent in the amount of about 7 parts by weight to 9 parts by weight; and

(e) water in the amount of about 75 parts by weight to about 85 parts by weight.

10. A coating composition as claimed in Claim 9 wherein said white cement includes:

(a) a high-early strength white cement in the amount of about 17 parts by weight to about 21 parts by weight; and

(b) a white waterproof cement in an amount of about 17 parts by weight to about 21 parts by weight.

11. A coating composition as claimed in Claim 9 further including a setting agent in the amount of about  $\frac{1}{16}$  parts by weight to about  $\frac{1}{8}$  parts by weight, the specific amount of said setting agent being approximately  $\frac{1}{16}$  part by weight for each 10% of relative humidity taken at the specific time and location of use.

#### References Cited

#### UNITED STATES PATENTS

|           |        |                |       |        |
|-----------|--------|----------------|-------|--------|
| 2,092,838 | 9/1937 | Gardner        | ----- | 106-97 |
| 2,929,729 | 3/1960 | Waggoner       | ----- | 106-89 |
| 3,102,039 | 8/1963 | Manecke        | ----- | 106-97 |
| 3,240,736 | 3/1966 | Beckwith       | ----- | 106-97 |
| 3,666,509 | 5/1972 | Horwitz        | ----- | 106-97 |
| 3,795,721 | 3/1974 | Gilbert et al. | ----- | 106-89 |
| 2,991,186 | 7/1961 | Furlan         | ----- | 106-98 |

DELBERT E. GANTZ, Primary Examiner

J. W. HELLWEGE, Assistant Examiner

U.S. Cl. X.R.

30 106-97